

May 8, 1945.

E. O. KALIL ET AL

2,375,742

PHOTOGRAPHIC FLASH LAMP

Filed Sept. 30, 1942



Fig.2.

Fig.1.



Fig.3.

INVENTORS.  
Emil O. Kalil &  
BY William S. Gleim.  
Leway & Witter atty.

## UNITED STATES PATENT OFFICE

2,375,742

## PHOTOGRAPHIC FLASH LAMP

Emil O. Kalil, Brooklyn, N. Y., and William E. Gleim, Bloomfield, N. J., assignors to Wabash Appliance Corporation, Brooklyn, N. Y., a corporation of New York

Application September 30, 1942, Serial No. 460,222

7 Claims. (Cl. 67—31)

This invention consists in a new and improved photographic flash lamp having certain advantages over those heretofore known and employing in its construction novel compositions of combustible materials not heretofore used for the generation of light in such lamps.

Uniform performance and reliability are the most important characteristics of flash lamps. Not only must the flash always reach the same high intensity of light, but it must follow dependably a predetermined time curve so that it may be synchronized with the opening of the camera shutter or other moving object. Moreover it is desirable that the time curve should provide an appreciable build-up interval before the maximum intensity of the flash is reached, in order, for example, to allow for actual shutter movement.

The combustible or ignitable material of the lamp must be such that it may be readily and instantaneously ignited or primed by the limited energy of a flash light battery, that it be capable of generating a flash of high intensity and that its functions should be properly carried out without danger of explosion or formation of toxic gases.

We have discovered that all these desirable results and others that will be hereinafter pointed out may be achieved by properly locating and exposing an area of zirconium within an oxygen-filled bulb in proximity to an igniting device responsive to the passage of an electric current. In the best form now known to us a paste of finely divided zirconium powder is mixed with a small amount of a powdered oxidizing ingredient and then this paste is spread as a coating upon any suitable supporting or carrying medium in the bulb. The supporting medium may be of any desired shape, but is preferably symmetrical with respect to the bulb, as for example, a ring or collar disposed concentrically in the axis of the bulb.

In preparing zirconium for this use, it is desirable to reduce the commercially available black or black-grey zirconium powder to a finer state of subdivision, as by ball milling for several hours, in general controlling the action of the combustible mixture by regulating the particle size of the metal powder, and then converting it to the form of paste by adding any suitable binder as nitro-cellulose, gum arabic, or shellac n solution.

The fulminating or oxidizing agent may take the form of potassium perchlorate, (KClO<sub>4</sub>), NaClO<sub>3</sub>, PbO<sub>2</sub>, CaO<sub>2</sub> or MgO<sub>2</sub>, NH<sub>4</sub>NO<sub>3</sub>, PbN<sub>6</sub>,

BaN<sub>6</sub>, or any equivalent oxide or fulminating mixture, and by varying the proportions of these agents the shape of the time curve of the lamp may be controlled and the point of maximum intensity of the flash may be advanced or delayed as desired for the requirements of the lamp manufactured.

While all the oxides mentioned are satisfactory, certain of them give up their oxygen at a relatively slower rate than others. For example, the greater the proportion of MgO<sub>2</sub> in the paste, the more delayed will be the instant of maximum light intensity of the flash. Preferably and as herein shown the lamp may include an igniting area of relatively slow burning composition leading to a substantial area of relatively fast burning composition.

The major part of the oxygen for combustion is supplied by filling the bulb with oxygen or other oxygenous gas. Under these conditions the percentage of oxidizing ingredient in the combustible paste is critical. The optimum conditions are such that the zirconium particles should be blasted from their supporting medium into the oxygen atmosphere of the bulb in very finely divided form, approaching a colloidal dispersion in the oxygen, and burn rapidly totally surrounded by oxygen before they strike the wall of the bulb. Accordingly sufficient KClO<sub>4</sub> or the like is added to start the reaction of combustion and to insure removal of the combustible paste from its support and the desired dispersion. 2% to 5% by weight of oxidizer or fulminator results in a very satisfactory mixture. Should the percentage be increased beyond 6% or 7% there is a marked decrease in light for two reasons. Oxidizer present above 5% practically blasts the zirconium directly against the side walls of the bulb. Consequently it does not have time to burn completely and in addition to the loss of light output the walls of the bulb are blackened and a substantial amount of light is lost on that account. By holding the oxidizer or fulminator at or below 5% this excessive blasting effect and blackening of the bulb are both eliminated and a satisfactory time curve is secured.

Zirconium is one of a group of metals which burn freely in oxygen giving off actinic light, and is the best of these metals now known to me for purposes of this invention. However, Al, Mg, and alloys thereof have substantially the same properties and may be regarded as equivalent to zirconium when used as a substitute for it in the manner above explained.

These and other features of the invention will

be best understood and appreciated from the following description of a preferred embodiment thereof, selected for purposes of illustration and shown in the accompanying drawing in which,

Fig. 1 is a view in perspective of the completed lamp,

Fig. 2 is a fragmentary view on an enlarged scale showing the disposition of the combustible material in the lamp, and

Fig. 3 is a characteristic time curve of a lamp of my invention.

The flash lamp herein shown comprises a glass bulb 10 and metal base 11 which may be of any desired commercial shape and size. Within the bulb is located the mount comprising the glass stem 12 in which are sealed leads 13. To these are welded extensions of nickel wire offset toward each other above the end of the stem and brought into close proximity and parallel relation at their upper ends. Between these two ends extends a fine filament 15 of such characteristics that it fuses readily in transmitting a low voltage current. Upon the ends of the nickel extension wires 14 are placed beads 16 of ignitable priming or fulminating compound. The composition of these priming beads consists in zirconium powder prepared as above outlined, blended with  $KClO_4$  and  $MgO_2$  or equivalent oxidizers in proportions approximating

|           | Per cent |
|-----------|----------|
| Zirconium | 90       |
| $KClO_4$  | 2        |
| $MgO_2$   | 8        |

In these beads therefore the slower oxidizer  $MgO_2$  predominates and the composition is relatively slow burning on this account although well adapted to serve as a priming compound.

As herein shown the combustible light source material is distributed within the bulb upon a ring-shaped supporting medium disposed substantially concentrically with respect to the priming beads and to the bulb, in a plane substantially level with the priming beads. The supporting ring may be made out of nickel wire or other suitable metal and mounted in the lamp by means of an angle wire 17 which is herein shown as welded to one of the extension wires 14. The ring itself is completely encased in a coating 18 of a paste of zirconium,  $KClO_4$  and  $MgO_2$  in approximately the following proportion:

|           | Per cent |
|-----------|----------|
| Zirconium | 95       |
| $KClO_4$  | 3.75     |
| $MgO_2$   | 1.25     |

These dry ingredients may be mixed in paste form with a liquid binder and the paste applied to the ring by dipping it one or more times below the surface of the paste, and when the paste dries it constitutes a firm coating which may be handled with convenience in the manufacture of the lamp. 250 mg. of a paste having the above formula will produce approximately 30,000 lumen-seconds, when flashed in an atmosphere of oxygen at 550 mm. pressure of mercury.

It will be apparent that the priming charge and the flash composition are supported as distinct masses freely exposed to the oxygen atmosphere of the bulb.

In operation the filament 15 is fused by closing a circuit through the leads of the lamp. The priming beads 16 are immediately ignited and within a few milliseconds the coating 18 of the ring is uniformly ignited from the burning beads. The faster burning coating is exploded

to the extent of blasting the zirconium particles it contains into the oxygen atmosphere of the bulb wherein they burn rapidly with the emission of actinic light.

5 A typical curve illustrating the action of the lamp is shown in Fig. 3 from which it will be noted that about five milliseconds is consumed in the fusion of the filament 15 followed by about seven milliseconds for the combustion of the priming beads 16. Combustion of the coating material begins at about the twelve millisecond point and the light intensity runs up on a very steep curve to a maximum of about 1,000,000 lumens at the twenty millisecond mark. From 10 then on the light intensity falls off on a gradual curve to the sixty-five millisecond point. It will be understood, of course, that the character of this curve may be varied substantially by varying the composition and amount of the priming beads and combustible ring coating. For example, the build-up time may be decreased by increasing the percentage of  $KClO_4$  at the expense of the percentage of  $MgO_2$  in the priming beads.

15 The flash lamp herein described represents the most desirable embodiment of the invention now known to me but may be varied in many of its details within the scope of the invention. While the lead extensions and ring have been described as of nickel it is entirely practicable to employ iron or ferrous alloys. Where metal is used it is desirable to keep the wire diameter of the ring small so that the ring shall not absorb heat and so lower the lighting efficiency of the compound. The composition of the priming and light source 20 paste has been stated as best adapted for a lamp flashing in accordance with the specific curve of Fig. 3 and, of course, if a different curve is desired the composition may be correspondingly varied in the manner above suggested.

25 40 While we prefer to employ priming or igniting beads having oxidizing ingredients it is necessary for purposes of our invention only that we have available fulminating material generating sufficient heat to ignite the combustible light-generating material upon the supporting medium and for 45 this function barium azide or lead azide are acceptable agents.

45 It will be understood that there are two distinct phases in the action of the lamp of our invention: first, driving the combustible material out into the oxygen atmosphere of the bulb quickly, faster than the rate of flame propagations and in very finely dispersed form, and 50 second, burning the oxygen-surrounded particles before they become plastered on the walls of the bulb. This, of course, requires a fine balance of the ingredients used and can be effected only between critical limits. These limits may be stated as 80-97% zirconium to 20-3% fulminating ingredients.

55 60 Having thus disclosed our invention and described in detail an illustrative embodiment thereof, we claim as new and desire to secure by Letters Patent:

65 70 75 1. A photographic flash lamp having a gas-filled bulb containing an ignitable primer adapted to be detonated by an electric current, a ring located concentrically within the bulb and in proximity to said primer and having a coating of powdered zirconium mixed with a fulminating agent in proportions between 80-97% zirconium to 20 to 3% fulminating agent, the said primer and zirconium coated ring being supported separately and freely in the gaseous atmosphere of the bulb.

2. A photographic flash lamp having an oxygen-filled bulb containing an ignitable primer and a carrier exposing in the bulb and adjacent to the primer a substantial area of zirconium mixed with  $KClO_4$  and  $MgO_2$  in proportions between 80-97% zirconium to 20 to 3%  $KClO_4$  and  $MgO_2$ , the said zirconium mixture being supported freely in the oxygen atmosphere of the bulb.

3. A photographic flash lamp having an oxygen-filled bulb containing an ignitable primer and a carrier exposing adjacent to the primer a substantial area of zirconium mixed with an oxidizing agent comprising about 75 parts  $KClO_4$  and about 25 parts  $MgO_2$ , the said zirconium mixture being supported freely in the oxygen atmosphere of the bulb.

4. A photographic flash lamp having an oxygen-filled bulb containing a fusible filament, a carrier exposing a substantial area of zirconium mixed with an oxidizing agent containing a high proportion of  $KClO_4$  and a lower proportion of  $MgO_2$ , and an ignitable primer interposed between said fusible filament and carrier and comprising a high proportion of  $MgO_2$  and a lower proportion of  $KClO_4$ , said primer and zirconium mixture being supported separately in the oxygen atmosphere of the bulb.

5. A photographic flash lamp comprising an oxygen-filled bulb having an ignitable primer

therein, and a supporting medium adjacent to the primer coated with a dried paste having a composition approximating Zr 95%,  $KClO_4$  3.75% and  $MgO_2$  1.25%, said primer and said paste being separately supported in the oxygen atmosphere of the bulb.

6. A photographic flash lamp comprising an oxygen-filled bulb having leads therein supporting an ignitable priming charge having a composition approximately Zr 90%,  $KClO_4$  2%,  $MgO_2$  8%, and a supporting ring disposed symmetrically in the bulb adjacent to the priming charge and having a coating of dried paste of a composition approximately 95% zirconium in finely divided powder, 3.75% potassium perchlorate and 1.25% magnesium dioxide, the priming charge and the paste composition of the said ring being disposed as distinct masses in the oxygen atmosphere of the bulb.

7. In a photographic flash lamp, supplementary light sources comprising a body comprising approximately Zr 90%,  $KClO_4$  2% and  $MgO_2$ , and a second body comprising approximately Zr 95%,  $KClO_4$  4% and  $MgO_2$ , the two bodies being supported as distinct masses and freely exposed within the lamp.

EMIL O. KALIL,  
WILLIAM E. GLEIM.